

## [54] APPARATUS FOR MANUFACTURING FINE METALLIC FILAMENTS

[75] Inventors: Yoshiyuki Tada; Hideo Ogita; Takeshi Yoda, all of Itami, Japan

[73] Assignee: Sumitomo Electric Industries, Ltd., Osaka, Japan

[22] Filed: Oct. 16, 1973

[21] Appl. No.: 406,987

## Related U.S. Application Data

[62] Division of Ser. No. 254,124, May 17, 1972, Pat. No. 3,785,036.

## [30] Foreign Application Priority Data

May 17, 1971 Japan..... 46-33080

[52] U.S. Cl. .... 29/200 B, 29/200 D, 29/413, 29/419

[51] Int. Cl. .... B23p 19/00, B23p 19/04

[58] Field of Search..... 29/200 D, 200 B, 413, 419

## [56] References Cited

## UNITED STATES PATENTS

3,254,396 6/1966 Mushey..... 29/413  
3,337,944 8/1967 Morris ..... 29/413

Primary Examiner—Thomas H. Eager  
 Attorney, Agent, or Firm—Sughrue, Rothwell, Mion,  
 Zinn & Macpeak

## [57] ABSTRACT

Apparatus for producing fine metallic filaments which comprises:

supply means for supplying a drawn composite wire comprising a bundle of a plurality of metallic filaments surrounded by an outer metal tube; cutting means comprising cutting bites arranged symmetrically with respect to the composite wire in the cutting means for cutting and removing most of the outer metal tube of the composite wire on opposite sides of the metal tube; rolling means comprising oppositely disposed rolls for pressing the uncut sides of the composite wire and to cause the composite wire to be compressed and spread outwardly in a direction perpendicular to the cut sides of the metal tube and for causing the metal tube to divide at the cut surface; and pickup means for taking up the divided parts of the metal tube and the metallic filaments.

4 Claims, 6 Drawing Figures



PATENTED OCT 1 1974

3,838,488

**FIG 1**



**FIG 2**



**FIG 3**



**FIG 4**



**FIG 6**



**FIG 5**

## APPARATUS FOR MANUFACTURING FINE METALLIC FILAMENTS

This is a division of U.S. Pat. No. 3,785,036 Tada et al., issued Jan. 15, 1974 from an application filed May 17, 1972, Ser. No. 254,124.

### BACKGROUND OF THE INVENTION

#### 1. Field of the Invention

This invention relates to apparatus for producing a yarn of fine metallic filaments at low cost, and especially to a novel apparatus of producing a yarn of fine metallic filaments by bundle drawing wherein the outer metal tube of a composite wire is mechanically separated from core filaments present inside the outer tube.

#### 2. Description of the Prior Art

In recent years, fine metallic wires about 0.150 to 0.005 mm in diameter made of carbon steel, alloy steel, stainless steel, etc. or yarns or slivers thereof have found applications as tire cords, metallic fibers for blending purposes, or fine metallic fibers for filters, etc. Generally, in the single wire drawing process using a die, the production of fine metallic filaments must be performed by the repetition of heat-treatments and drawings, and the productivity is low. This leads to an extreme increase in the cost of production. In an attempt to overcome these disadvantages, the bundle drawing process was devised, and has been utilized to some extent.

The conventional bundle drawing method comprises first coating the surfaces of material wires with a separator such as a metal oxide, graphite or an oil, which prevents the metallic bonding of the wires during the drawing and heat-treatment operations, or with a different metal by, for example, plating; inserting a bundle of a plurality of such material wires in a tube of a different metal, or covering this bundle of wires with a metallic tape at its outer circumference, and welding the seam portion thereby to form a composite wire; subjecting the composite wire to a diameter reduction treatment by drawing, and heat-treatment, etc. until the diameter of each filament reaches a certain desired value; and thereafter, dissolving the outer metal tube alone or together with the coated metal by a chemical method, and separating them from the core filaments, thereby obtaining fine metallic filaments.

According to this prior art method, the outer metal tube (A) alone or together with the coated metal (B) should be dissolved by dipping or electrolysis using a specially selected reagent solution which does not react with the fine metallic filaments present inside the tube, but reacts only with (A) or with (A) and (B) (A and B may be the same kind of metal). This dissolving operation generally takes a long time and requires strict control of the conditions. Furthermore, because of using a special chemical solution, the cost of production increases, and the recovery of the dissolved metal is difficult.

Accordingly, an object of this invention is to provide apparatus for producing fine metallic filaments by the bundle drawing method wherein the separation of the outer metal tube of the drawn composite wire is effected by a mechanical procedure instead of the conventional chemical procedure, whereby the above-mentioned defects of the prior art can be removed, and the separation treatment of the fine metallic filaments of the composite wire can be performed by a simple ap-

paratus within a shorter time, which reduces the cost of production, and whereby the recovery of the outer tube metal can be simultaneously performed in situ.

Another object of this invention is to provide apparatus for producing fine metallic filaments wherein by the mechanical procedure used for the separation treatment instead of the chemical procedure, the fine metallic filaments do not undergo corrosion, and products of good quality without breakage or deterioration in properties can be obtained.

### SUMMARY OF THE INVENTION

According to this invention, there is provided apparatus for producing fine metallic filaments by the bundle drawing method, wherein in order to separate the outer tube metal of the final drawn composite wire from the core filaments therein, the outer tube metal on both sides of the composite wire is cut near to the core filaments, and then both uncut surfaces of the composite wire are lightly rolled thereby to divide the composite wire continuously and thus form fine metallic filaments.

The apparatus of the present invention for producing fine metallic filaments comprises:

15 supply means for supplying a drawn composite wire comprising a bundle of a plurality of metal filaments surrounded by an outer metal tube,  
20 cutting means comprising cutting bites arranged symmetrically in relation to said composite wire in said cutting means for cutting and removing most of said outer metal tube of said composite wire on opposite sides of said metal tube,  
25 cutting means comprising cutting bites arranged symmetrically in relation to said composite wire in said cutting means for cutting and removing most of said outer metal tube of said composite wire on opposite sides of said metal tube,  
30 rolling means comprising oppositely disposed rolls for pressing the uncut sides of said composite wire, causing said composite wire to be compressed and to spread outwardly in a direction perpendicular to said cut sides of said metal tube and said metal tube to divide at said cut surfaces, and  
35 take-up means for taking up the divided parts of said metal tube and said metallic filaments.

The above and other objects of this invention along with the features and advantages thereof will become fully apparent as the description proceeds with reference to the accompanying drawings. Some embodiments of the present invention are illustrated in the drawings, but the invention is in no way limited thereto.

### BRIEF DESCRIPTION OF THE DRAWINGS

FIGS. 1, 2, 3 and 4 show one example of the process of producing fine metallic filaments in accordance with this invention, FIG. 1 showing a composite wire before drawing, FIG. 2 the composite wire after drawing, FIG. 3 the composite wire after cutting of both sides of the outer tube, and FIG. 4 fine metallic filaments finally obtained.

FIG. 5 is a schematic view of an apparatus to be used for the performance of the present invention to separate the outer tube metal of the drawn composite wire from the core filaments therein; and

FIG. 6 is a sectional view showing the state of cutting the outer tube metal in the apparatus shown in FIG. 5.

### DESCRIPTION OF THE PREFERRED EMBODIMENTS

In accordance with this invention, as shown in FIG.

1 same as in the above-described conventional method, a separator 2 is coated on the surfaces of material wires 1, or a different metal 2 is coated thereon by, for example, plating. A bundle of a plurality of the coated material wires is inserted in a tube 3 of a different metal, or the bundle of the material wires is covered with a metallic tape 3 at its outer circumference, followed by welding the seam portion to form a composite wire 4. The separator or metal coated layer 2 on the surfaces of the material wires is not altogether necessary when the material wires are not heat-treated in any subsequent step. Then, the composite wire obtained is subjected to a diameter reduction treatment by drawing, heat-treatment, etc. until the diameter of each core metallic wire 1 reaches a desired value, and a composite wire having the section as shown in FIG. 2 is obtained. The drawn composite wire is subsequently processed by an apparatus of the type shown in FIG. 5. Referring to FIG. 5, the reference numeral 4 represents a drawn composite wire including, for example, 91 high carbon steel filaments with a diameter of 0.050 mm and a mild steel tube having a thickness of 35 to 40 micrometers covering the outer circumference of a bundle of the steel filaments. A supply reel for the composite wire 4 is shown at 5. The composite wire 4 is passed through an outer tube cutting device 6, and drawn out. The drawing force is imparted by rolls 8 or a capstan (not shown) disposed between 6 and 7. This device 6 consists of two cutting bites 14 arranged symmetrically to each other as shown in FIG. 6, and is adapted to cut the outer metal 3 on both sides of the composite wire near to core filaments 1 inside the outer tube so that the composite wire has a section as shown in FIG. 3. The outer tube metal is cut to an extent as close as possible to the core filaments but without exposing the filaments even at points 3" which are the deepest cuts. For example, when the thickness of the composite wire between the cut surfaces is 0.48 mm, a layer of the outer metal tube having a thickness of 0.010 to 0.015 mm remains.

The composite wire 4' in which the outer layer on both sides have been cut is rolled by rolls 8 slightly to press the upper and lower uncut surfaces. At this time, it is necessary to provide a guide 7 which prevents the composite wire 4' from tumbling down towards the entry side of rolls 8.

By this rolling, the composite wire is collapsed upwards and downwards, and tends to spread laterally and become a flat wire. Since the surfaces of the core filaments have previously been coated with a separator such as metal oxides, graphite or metal soap, the filaments slip over each other, and are not deformed plastically. Hence, this stress inducing the lateral spreading to form a flat wire is concentrated on the thinnest points 3" of the outer metal as shown in FIG. 3, and these points are broken. Thus, by the rolling operation, the outer tube metal is divided into the upper and lower portions 3' and 3' and is separated from the core filaments 1'. If the rolling force at this time is excessive, the core filaments are plastically deformed to collapse. If, on the other hand, the rolling force is small, the continuous break of the outer tube metal does not occur. Therefore, the rolling conditions should be determined optionally by experiments in relation to the cutting conditions in the previous step.

The two divided outer metal portions 3' and a filament yarn 1' are separated by separating guide rolls 9

into a yarn of fine metallic filaments 1' and two outer metal portions 3', and coiled up by take-up reels 11, 12 and 13. The yarn of fine metallic filaments 1' thus taken up is in the state of being completely separated into the individual filaments as shown in FIG. 4. This is due to the effect of the separator pre-coated on the surfaces of the material wires.

A take-up device 10 having the take-up rolls 11, 12 and 13, for example, is of a slip-type take-up mechanism, or of a mechanism using a fixed torque motor, whereby the yarn and outer metals are coiled up in synchronous relationship with the speed of rolling while a certain prescribed tension is being imparted to the yarn and outer metal.

The above-described apparatus and method makes it possible to remove the outer tube metal from the composite wire containing fine metallic filaments therein by cutting and rolling and thus obtain a yarn of fine metallic filaments.

Since according to the present invention the separation treatment of fine metallic filaments in the bundle drawing method can be performed by a mechanical procedure using a simple apparatus without carrying out a troublesome and expensive chemical or electrochemical treatment, the operation is simple and the treatment time is short. Furthermore, because no cost is necessary for chemicals, the method has the advantage that the cost of production becomes lower. In the conventional method, the outer tube metal is dissolved in a chemical as a result of the chemical or electrochemical treatment, the recovery of the metal must be effected, for example, by electrolytic deposition or precipitation based on the formation of hydroxides, and therefore, generally becomes difficult and expensive. By contrast, in the present invention, it can be recovered as metal quite simply. Hence, when an especially expensive metal such as copper or nickel is used as the outer tube metal, the cost of production can be greatly curtailed.

The invention will now be illustrated further by the following examples.

#### EXAMPLE 1

Final composite wire

Outer tube metal: mild steel

Fine filament: 0.8 percent carbon steel

Diameter of the composite wire: 0.60 mm

Diameter of each filament (average): 0.050 mm

Number of filaments: 91

Thickness of the tube (average): 0.060 mm

Separator on the filament surfaces: talcum powder

The composite wire shown above was processed by an apparatus of the type shown in FIG. 5. The outer tube metal of the composite wire was cut continuously with application of a cutting oil so that the cut margin became 0.035 to 0.040 mm. Subsequently, the wire was slightly rolled by six high rolls in which the diameter of the working roll was 30 mm, and the outer tube metal was divided into two portions. These divided portions and a yarn of the fine metallic filaments therein were separately taken up. A yarn of 91 fine metallic filaments with a diameter of 0.05 mm was continuously obtained at a speed of 100 m/min.

#### EXAMPLE 2

Final Composite wire

Outer tube metal: mild steel

Final filament: 304 type stainless steel  
 Diameter of the composite wire: 0.71 mm  
 Diameter of each filament (average): 0.035 mm  
 Number of filaments: 300

Thickness of the tube (average): 0.050 mm  
 Separator on the filament surface: talcum powder

The composite wire shown above was cut by the same apparatus and method as used in Example 1 except that the cut margin was 0.020 to 0.025 mm. The subsequent procedure was the same as in Example 1, and a yarn of 300 fine metallic filaments having a diameter of 0.035 mm was obtained at a speed of 100 m/min.

We claim:

1. An apparatus for producing fine metallic filaments comprising  
 supply means for supplying a drawn composite wire comprising a bundle of a plurality of metallic filaments surrounded by an outer metal tube,  
 cutting means comprising cutting bites arranged symmetrically in relation to said composite wire in said cutting means for cutting and removing most of said outer metal tube of said composite wire on opposite sides of said metal tube,  
 rolling means comprising oppositely disposed rolls for pressing the uncut sides of said composite wire, causing said composite wire to be compressed and

to spread outwardly in a direction perpendicular to said cut sides of said metal tube and said metal tube to divide at said cut surfaces, and take-up means for taking up the divided parts of said metal tube and said metallic filaments.

2. The apparatus of claim 1, comprising additionally friction rolls or a drive-type capstan disposed between said rolling means and said cutting means, around which said composite wire is wrapped a few turns for drawing said composite wire through said cutting means.

3. The apparatus of claim 1, wherein a tumble-preventing guide is disposed at the entry side of said rolling means, said guide being adapted to press the cut surface of the composite wire lightly so as to position the cut surface of said composite wire always at right angles to the surfaces of the rolls upon entry of the composite wire between the rolls.

4. The apparatus of claim 1, wherein said take-up means for the divided portions of the outer tube metal and the metallic filaments comprises a slip mechanism or a fixed torque motor in synchronous relation to the speed of said composite wire passing said rolling means, said composite wire being under a certain prescribed tension.

\* \* \* \* \*